

Patented Oct. 17, 1922.

## UNITED STATES PATENT OFFICE.

WILHELM DIETERLE, OF FEUERBACH, NEAR STUTTGART, GERMANY.

## PHOTOGRAPHIC DEVELOPER.

No Drawing.

Application filed March 25, 1921. Serial No. 455,491.

*To all whom it may concern:*

Be it known that I, WILHELM DIETERLE, a subject of the Republic of Wurtemberg, in Germany, residing at Feuerbach, near Stuttgart, Germany, have invented certain new and useful Improvements in Photographic Developers (for which I have filed applications in Germany, patent issued under No. 327,111, filed on Oct. 24, 1918; additional patent issued under No. 328,617, filed on Dec. 10, 1918; additional patent issued under No. 333,687, filed April 18, 1920; Austria application filed Oct. 14, 1920; Switzerland application G 7695 filed on Aug. 18, 1920; France application 134,932 filed Oct. 11, 1920; Belgium application 232,860 filed Sept. 25, 1920; Italy application 39750 filed Sept. 10, 1920; Czechoslovakia application P 7680 filed Sept. 29, 1920; Sweden application No. 4614 filed Sept. 11, 1920; England application 32883 filed Nov. 22, 1920), of which the following is a specification.

In the course of experiments to determine the influence of substitutes for the nucleus or basic constituent of the familiar amido-phenol or amidocresol-developers on their developing properties, I have discovered that the accession of the carboxyl group and of the sulpho-acid group completely nullifies the developing capacity of the basic substances so long as the operations are carried out, according to the known practice, with sodium sulphite and sodium carbonate or potassium carbonate. By dissolving the developer in water and adding potassium carbonate, the carboxyl- and sulpho-acid groups are certainly converted into their alkaline salts, but this procedure does not result in the production of a developing solution. In order to restore the solutions containing carboxyls or sulpho-acids their original developing properties, the hydroxyl-groups are, according to this invention, also more or less completely converted into their alkaline salts by the application of free caustic alkali. Only thereupon are the developing properties, which the presence of the carboxyl- or sulpho-acid-groups had nullified, again restored, but they are then re-established in a radically different manner and, as it were, in an improved degree as is hereinafter mentioned. If only a part of the hydroxyl groups present, say 25%,

be neutralized with free alkali, a slow acting developer is produced, whilst, if on the other hand, say 50% of the hydroxyl groups present be neutralized, the developer produced is normal in its action, while the complete neutralization of the hydroxyl groups serves to impart to the developer the characteristic of rapid action. Broadly speaking, therefore, the carboxyl- or the sulpho-acid group forms, in a certain sense, a means of predetermining and regulating the developing properties of the solution as regards their speed of action.

Moreover, seeing that other favourable qualities from the point of view of technical photography are attained, the accession of the hydroxyl- or sulpho-acid groups produces valuable advantages and constitutes a great advance in relation to the developers hitherto made use of. Particularly is this the case as regards the power of my improved developers of compensating for the most diverse defects of exposure, more particularly for highly excessive exposure which may now be allowed to mount to several hundred-fold of the normal. These are advantages affecting the tyro, the skilled amateur or the professional photographer, for even the former, however defective the exposure, may still obtain reasonably satisfactory effects which, with any other developers, would infallibly have resulted in unmarketable goods, whilst the latter will be able to cope with problems in photography, which, with the resources hitherto at his disposal, were utterly insoluble.

Further advantages in technical photography are attained by the use of this invention: For example, my improved developers show no tendency to indistinct or foggy effects, not even to the yellow stain hitherto invariably resulting from prolonged development. The negatives may be reduced in the usual manner, by ammonium persulphate. According to the degree of dilution of the developing solution, the silver precipitate exhibits a colour varying from black to brown, a special valuable property for diapositive photographs or those taken by gas-light. Potassium bromide furnishes an extensive scale of reducing when used with my improved developers. The latter cause no discolouration of the hands and possess all the advantages and none of the disad-

vantages of the popular pyrogallol developers.

The following examples are taken from the amidosalicylic acids treated with hydrochloric acid:

A stock solution of hydrochlorated amidosalicylic-acid of a two- or three-fold degree on concentration may be prepared in the following proportions:

|    |                                                                       |          |
|----|-----------------------------------------------------------------------|----------|
| 10 | Hydrochlorated paramidosalicylic-acid                                 | 100 gm.  |
|    | Sodium sulphite, free from water                                      | 500 gm.  |
|    | Normal (i.e. 5-fold strength) (200 gms. sodium hydrate—NaOH—in liter) | 210 cc.  |
|    | Water                                                                 | 4790 cc. |

Five litres of a stock solution (5) which may be preserved indefinitely, are thus produced. For developing purposes this solution is diluted with an equal or up to a double volume of water and then reacted on, according to requirements with the following proportions of ordinary sodium hydrate solution:

- Solution 1. For an illumination above the average and for slow action: S. 50 cc.; aq. 50 cc.; 1/n NaOH 3 cc. 1/n NaOH represents a solution of 40 gms. NaOH in a liter of water.
2. For a normal illumination and quicker action: S. 50 cc. aq. 50 cc. 1/n NaOH 5 cc.
  3. For a normal illumination, and rapid action: S. 50 cc. aq. 50 cc. 1/n NaOH 7 cc.
  4. For a sparse illumination and rapid action: S. 50 cc. aq. 50 cc. 1/n NaOH 8 cc.
  5. For enlargements; with normal action: S. 50 cc. aq. 50 cc. 1/n NaOH 10 cc.
  6. For enlargements; with quick action: S. 50 cc. aq. 50 cc. 1/n NaOH 12 cc.

According to requirements, these proportions may be still further varied for special purposes. If the solution (5) be, for example, more strongly diluted the result is a slower development with brown tones. From gradual neutralization, after re-

peated developing, the sodium hydrate becomes exhausted of its reactive properties and must, therefore, be restored by addition from time to time, so that the developing solution may recover its original efficacy.

The sodium hydrate is neutralized, i. e., converted into sodium carbonate and carbonate of soda and, consequently, made inefficient by the bromic hydracid, which is created during the process of the development, as well as by the carbonic acid of the air. This neutralization of the sodium hydrate goes on much more rapidly than the consumption of the amidosalicylic acid by the development itself. It is for this reason that the developer may repeatedly be regenerated through the addition of sodium hydrate, until it will gradually become inefficient through continued use.

Having now particularly described and ascertained the nature of my invention and in what manner the same is to be performed, I claim:

1. A photographic developer consisting of a sulpho-acid of an amidophenol derivative in caustic alkali solution.

2. A photographic developer consisting of the carbo- and sulpho-acids of an amidophenol or a homologue of the same in caustic alkali solution.

In testimony whereof I affix my signature in presence of two witnesses.

DR. WILHELM DIETERLE.

Witnesses.

E. SCHLEICHER,  
FRIEDA KLAIBES.